

J. Reichenbach.

Making Chilled Castings.

No. 89,070.

Patented Apr. 20, 1869.

Fig. 1.



Fig. 3.



Fig. 2.



Witnesses.

George B. Cushing.

Thos. B. Kerr.

Inventor.

John Reichenbach,  
by Bakewell & Christy,  
his Atty's.



JOHN REICHENBACH, OF ALLEGHENY CITY, PENNSYLVANIA, ASSIGNOR TO HIMSELF,  
JOHN HEATH, AND WILLIAM R. FITZSIMONS, OF SAME PLACE.

Letters Patent No. 89,076, dated April 20, 1869.

**COMPOSITION FOR MAKING CHILLED CASTINGS.**

The Schedule referred to in these Letters Patent and making part of the same.

*To all whom it may concern:*

Be it known that I, JOHN REICHENBACH, of Allegheny City, in the county of Allegheny, and State of Pennsylvania, have invented a new and useful Improvement in Mixture for Chilled Castings; and I do hereby declare the following to be a full, clear, and exact description thereof, reference being had to the accompanying drawing, making a part of this specification, in which—

Figure 1 is a cross-section of a flask, in which is a series of moulds for casting nuts, with chills in place for forming the threaded eye in each of the nuts;

Figure 2 is a side view of a threaded metallic chill; and

Figure 3 is a section of a cast-metal nut, as formed by a plane passing longitudinally along the axis of the eye of the nut.

In making chilled casting heretofore, it has generally been found necessary to remove the casting from the chill as soon as the metal was fairly set, in order to prevent their becoming inseparably united, and this fact has rendered it impracticable to employ a chill in casting many articles; especially is this true in respect to all castings, where the chill cannot be immediately removed, as in castings in which a chilled face is desired on two or more sides, also in casting metal nuts with threaded chilled eyes, and in casting many other articles of like character.

My invention is designed to obviate this difficulty, and the nature of it consists in coating the chill before the casting is done, with a solution of gum-shellac, which, when dry, leaves a thin crust on the chill, against or on which to teem the molten metal.

To enable others skilled in the art to make use of my invention, I will proceed to describe it, and its manner of use, illustrating it more particularly by a description of its application to the casting of threaded nuts.

*a* is a threaded chill of the form of a screw, and *b* is a nut cast thereon.

The threaded chill *a*, I place centrally in a mould of the proper size and shape for forming the outer face of the nut, or more commonly arrange a number of such chills, one in each of a series of nut-moulds, *c*, as shown in fig. 1, in which *d* is the flask, and *f f'* the sand-mould.

The nuts, or patterns for forming the nut-moulds, or cavities *c*, are screwed on to the chills *a*, and the mould formed in the usual way, gates *e* and sprues *e* being made at the same time for the usual purposes.

Having then removed the upper part *f* of the mould, the nuts and chills *a* are taken out and the nuts screwed off.

The chills *a*, or so much of them as is to be exposed to the melted metal, are then coated with a mixture of gum-shellac, alcohol, and lamp-black.

In making the mixture, I take the ingredients named, in about the proportion of one-half pint of alcohol, one ounce gum-shellac, and a table-spoonful of lamp-black. The gum-shellac is dissolved in the alcohol, and the lamp-black is added.

This mixture being applied to the face of a chill, effectually prevents melted iron from forming a solid union therewith.

The chills *a* being coated with this mixture, they are replaced in the cavities *c*, the upper part *f* of the flask is replaced, and the casting proceeds.

The metal is turned in at one gate *e*, flows along the cavities *c*, through the sprues *e*, till all are full.

When it is "set," the cast nuts are removed, broken apart, turned off, each from its chill *a*, and thereby are produced nuts, each with a perfectly formed chilled threaded eye, as shown in section in fig. 3.

The mixture described, forms a thin crust on the face of the chill, the alcohol readily evaporating, and such crust so far resists the action of the heat of the melted metal, as to prevent the melted metal from forming a fixed union with the chill.

The same is true, even if the newly formed casting remain on or in contact with the chill till it is cold. It can still be easily removed.

In the application of the composition, or mixture described, I do not limit myself to the manufacture of nuts, but extend it to making all kinds of chilled castings.

The face of the chill against which the casting is to be done, is coated with the mixture described, with the result already stated.

If the castings to be made are large, I sometimes sprinkle a little sand on the chill after it is coated with this mixture, in order to give additional body to the coating, but in small castings, the gum-shellac and lamp-black give all the coating that is required.

In this way I am enabled to chill any or all faces of a casting, no matter how numerous they may be, or how irregular their forms, and can also produce chilled castings more economically since the work of casting need not be interrupted to remove the casting from its chill, lest the two form a solid union.

What I claim as my invention, and desire to secure by Letters Patent, is—

As a coating for the chill in making chilled castings, a mixture of gum-shellac, alcohol, and lamp-black, in the proportions, and used substantially as stated.

In testimony whereof, I, the said JOHN REICHENBACH, have hereunto set my hand.

JOHN REICHENBACH.

Witnesses:

A. S. NICHOLSON,  
G. H. CHRISTY.